

July 28, 1925.

1,547,877

F. KOLB

## METHOD AND APPARATUS FOR MAKING CONTINUOUS TIN FOIL

Filed Oct. 4, 1924

2 Sheets-Sheet 1



### Inventor

Fred Kalt

By Frank Thomas  
his Attorneys

July 28, 1925.

1,547,877

F. KOLB

# METHOD AND APPARATUS FOR MAKING CONTINUOUS TIN FOIL

Filed Oct. 4, 1924

2 Sheets-Sheet 2



Fred Kolb

By Frank O'Connel  
his Attorneys

Patented July 28, 1925.

1,547,877

# UNITED STATES PATENT OFFICE.

FRED KOLB, OF ST. LOUIS, MISSOURI.

## METHOD AND APPARATUS FOR MAKING CONTINUOUS TIN FOIL.

Application filed October 4, 1924. Serial No. 741,574.

To all whom it may concern:

Be it known that I, FRED KOLB, a citizen of the United States, residing at the city of St. Louis and State of Missouri, have invented certain new and useful Improvements in Methods and Apparatus for Making Continuous Tin Foil; and I do hereby declare the following to be a full, clear, and exact description of the same, reference being had 10 to the accompanying drawings, forming part of this specification.

This invention relates to a method of and apparatus for making tin foil and particularly to the making of a continuous sheet of such material.

While the primary object of the invention is the production of a continuous sheet of tin foil, another object contemplated is the provision of means for coating one side of the 20 lead core with a heavier layer of tin than that deposited on the other side.

With these and other objects in view, the invention consists in certain novel details of construction and combinations and arrangements of parts all as will hereinafter be more fully described and the novel features thereof particularly pointed out in the appended claims.

In the accompanying drawings,—

30 Figs. 1 and 1<sup>a</sup> jointly illustrate a side elevational view of the preferred form of apparatus embodying the invention of the instant case.

Fig. 2 is a detail view of a portion of the 35 means for giving the core a preliminary coating of tin.

Fig. 3 is a diagrammatic view of means for spraying the preliminarily coated core with the final coating of tin.

40 Fig. 4 is a longitudinal sectional view of spraying device for spraying the molten tin on the sheet.

Fig. 5 is a transverse sectional view of the structure shown in Fig. 4; and

45 Fig. 6 is a detail view of the edging rolls which govern the width of the finished product.

Fig. 7 is an end view of the structure 50 shown in Fig. 5, the view being taken in a direction opposite to that of the arrows used for indicating Fig. 6.

The first few steps in the method and apparatus contemplated by the present invention may be practiced with apparatus now in common use. For instance, the molten material, such as lead, which is to

constitute the core of the tin foil, is contained in a reservoir 10 from which it is regulably and constantly discharged onto an inclined table or platform 11 on which it 60 takes the form of a film or sheet. To aid in solidifying the core, the table 11 may be formed with interior passages for the circulation of any cooling medium such as water. As the sheet of lead, or other core 65 material, is drawn off the table 11, it passes between suitable sizing rolls 12 which may be provided in accordance with common practice, a scraper 13 being here shown at the discharge side of said rolls. After passing 70 beyond the scraper, the core is passed through two tanks 14, 15, the former containing the usual cleaning acid and the latter water for washing the core clean of the acid, suitable guides 16 being provided 75 in said tanks to insure the core being immersed. Both the bath of acid and of water may be maintained at the proper temperatures by heat applied thereto through the heating chambers 14<sup>a</sup>, 15<sup>a</sup>, and drains for 80 said tanks are also provided, as indicated at 17.

After coming out of the washing bath, the endless core passes into a bath of molten tin for the purpose of preliminarily coating both sides thereof. To secure proper submergence of the core in this bath of tin in the tank 18 vertically movable guides 19 are provided. Preferably guides 19 are supported from one end of cables 20, the cables 85 extending over pulleys 21 with their opposite ends each supporting a counterbalance 22. This permits the operator to raise and dip the endless core any number of times desired to give the core its proper preliminary coating. At the base of tank 18 there is formed a heating chamber 18<sup>a</sup> and within said tank, preferably at the 90 points where the core enters and leaves the bath, there are provided pipes 23 having orifices therein through which air under 95 pressure is forced for the purpose of preventing the accumulation of dross and dirt at these points in the bath.

After leaving the tank 18, the core, preliminarily coated, passes between two spraying devices 24 which deposit additional tin on the opposite sides of the core, this being the final coating step. As shown more in detail in Figs. 3 to 5 each sprayer consists 100 of a nozzle comprising an inner pipe 25 and a sleeve 26 concentrically arranged on 105

110

said pipe, there being openings such as longitudinally extending slots 27 in both the pipe and sleeve. The supply of tin is held in a tank 28 below the endless core and the 5 molten material is supplied to the pipes 25 by a cast iron gear pump 29 mounted in said tank.

To regulate the quantity of tin discharged from the spraying nozzle, each pipe is provided with a collar 30 and each sleeve with a collar 31, both collars having a forked arm or extension 32 which are alined with each other. In the fork of the collar on pipe 25 is a trunnion nut 33 and in the collar on 10 sleeve 26 there is a trunnion sleeve 34 on whose outer face is a dial 35 preferably marked with one hundred circularly arranged equi-distantly spaced graduations. Working in said nut and sleeve is a screw 36 held against total withdrawal of collars 37, 38 and on collar 38 there is a pointer 39 adapted to cooperate with the series of graduations on the trunnion sleeve. Sleeve 26 is loose on pipe 25 and by manipulating screw 15 36 the openings in said collar and sleeve can be so moved with respect to each other as to vary the size of the opening and thereby regulate the amount of molten tin discharged, as desired. As the regulation of 20 one nozzle is entirely independent of that of the other it is apparent that the amount of tin deposited on one side of the core can be varied from that deposited on the opposite side, thereby giving one side a heavier 25 coat than the other. This is an advantageous feature. To adapt the spraying nozzles to use on cores of different widths, longitudinally spaced rings 40 are provided on the nozzles, each carrying a strip 50 30 working in the slot in sleeve 26. The rings 40 are locked at any point on the nozzle by set screws but by loosening up the screws, the strips may be moved toward or away from each other to vary the length of the 35 slot as desired. The metal in tank 28 is heated from the combustion chamber 41 and suitable drains 42 and 43 are also provided for the two tanks of tin.

After leaving the spraying nozzles, the 40 fully coated core passes over a cooling table 44, similar to table 11, and from thence it passes through between edging rolls 45 at opposite edges of the core. These rolls 45 are preferably adjustable horizontally toward and away from each other to accommodate different width cores.

Beyond the edging rolls, the coated core is passed between suitable finishing rolls 46 which may be of any commercial form and 45 from these rolls the finished product is conveyed to a spool or winding roll 47 or other suitable place for storage.

What I claim is:

1. A continuous method of making tin foil which consists in forming a continuous

core of suitable material, passing it through cleaning and washing liquids, immersing said core to coat it with a preliminary deposit of tin, subsequently spraying a molten tin composition on opposite sides of said core to 70 give it the desired coating of tin, and finally passing said tin coated core through finishing rolls.

2. A continuous method of making tin foil which consists in forming a continuous 75 core of suitable material, passing said core through cleaning and washing tanks, depositing a preliminary coating of tin on opposite sides of the core, subsequently spraying molten tin composition on said core and 80 finally passing said tin coated core through finishing rolls.

3. A continuous method of making tin foil such as described in claim 2 characterized by regulating the final spraying of tin 85 on the core to deposit a heavier coating of tin on one side than on the other side.

4. A continuous method of making tin foil such as described in claim 2 characterized by regulating the final spraying of tin on the 90 core to deposit a heavier coating on one side than on the other and simultaneously spraying both sides of said core.

5. A continuous method of making tin foil which consists in forming a continuous core 95 of suitable material, passing it through cleaning and washing liquids, immersing said core to coat it with a preliminary deposit of tin, subsequently spraying a molten tin composition on opposite sides of said core to 100 give it the desired coating of tin, passing said tin coated core through edging rolls to determine the width of the finished product, and finally passing said tin coated core 105 through finishing rolls.

6. In an apparatus for continuously producing tin foil, the combination of a reservoir for the molten material forming the core of the finished product, a pouring plate or table, on which the molten material is deposited in film-like form, means for cooling the material as it passes over the table to form the core, sizing rolls, cleansing and washing receptacles through which the core passes, means for placing a preliminary deposit of tin on the core, means for subsequently spraying opposite sides of the core with a coating of tin, and finishing rolls through which the tin coated core is passed. 115

7. In an apparatus for making tin foil, a reservoir for a molten material from which a suitable core is formed, a cooling table over which said material is poured from said reservoir to form a continuous core, sizing rolls, and cleaning and washing tanks 125 through which said endless core passes, a preliminary bath of molten tin in which said endless core is immersed, means for subsequently spraying opposite sides of said core with a final coating of molten tin, and 130

finishing rolls through which said core with the final coating thereon is passed.

8. An apparatus such as set forth in claim 7, characterized by the provision of edging rolls intermediate the finishing rolls and the means for depositing the final coating of tin on the core.

9. An apparatus such as set forth in claim 7, characterized by the spraying means comprising a pair of concentrically arranged pipes having spraying orifices therein, a body of molten tin, a pump located in said tin connected with said pipes, and means for adjusting the concentrically arranged pipes one on the other to vary the size of said openings.

10. An apparatus such as described in claim 7, characterized by the spraying means

comprising a pair of concentrically arranged pipes on each side of the endless core and 20 each pair of pipes having discharge openings therein, a pump for supplying molten tin to each pair of pipes and separate means for regulating the discharge of molten tin from each pair of pipes whereby a heavier 25 coating of tin may be deposited on one side of the core than on the other.

11. An apparatus such as set forth in claim 6, characterized by the provision of a tank containing the tin used for preliminarily coating the core and means within said tank to prevent the accumulation of dross and dirt at the points where the core enters and leaves said tank. 30

FRED KOLB.